

## UNITED STATES PATENT OFFICE

2,127,564

## ZINC AMMONIUM CHLORIDE FLUXES

Raymond J. Kepfer, Lakewood, Ohio, assignor,  
by mesne assignments, to E. I. du Pont de Ne-  
mours & Company, Wilmington, Del., a cor-  
poration of Delaware

No Drawing. Application March 5, 1936,  
Serial No. 67,306

## 1 Claim. (Cl. 148-26)

This invention relates to zinc ammonium chlo-  
ride galvanizing fluxes, and is particularly directed  
to processes wherein unsatisfactory zinc am-  
monium chloride galvanizing fluxes are made  
5 suitable for use with foaming agents by reducing  
the amount of sulfates present as impurities.

In hot dip galvanizing, a bath of molten zinc  
is covered with a flux. As articles to be gal-  
vanized are lowered into the molten zinc bath they,  
10 of course, first pass thru the flux where they are  
cleaned and prepared for the reception of a metal  
coating.

It has heretofore been the practice to employ  
foaming agents such as glycerine, tallow, and soap  
15 bark with the flux in order to produce a foam or  
froth. Ordinarily the foaming agent and flux are  
separately added, as required, to the zinc bath.  
Sometimes the zinc ammonium chloride flux and  
foaming agent in predetermined proportions are  
20 simultaneously added to a zinc bath either by  
adding a mixture of flux and foaming agent di-  
rectly to the bath or by adding such a mixture to  
a pre-wash from which the metal being treated  
carries the flux and foaming agent to the bath.

25 The foam produced by means of foaming  
agents serves to entrap vapors and gases and to  
retard the rate of volatilization of the flux. For  
galvanizing operations of this type it is essential  
30 that the foam be satisfactory in character and of  
sufficient thickness.

Galvanizers have frequently been confronted  
with the difficulty that, for no apparent reason, it  
is sometimes extremely difficult or even impossible  
35 to obtain a satisfactory foam. Sometimes by  
using a great excess of foaming agent it was possi-  
ble to obtain a moderately satisfactory foam.  
In most instances, the difficulties were surmount-  
ed only by purchasing a new lot of zinc am-  
40 monium chloride flux which would not be so un-  
satisfactory.

I have found that this hitherto unaccountable  
behavior on the part of zinc ammonium chloride  
fluxes is attributable to the presence therein of an  
45 excess of sulfate. When sulfates are present in  
excess of about .2%  $SO_3$  in zinc ammonium  
chloride fluxes, it is difficult or impossible to  
produce a satisfactory foam by the use of the  
customary foaming agents even when such agents  
50 are used in very large amounts. Without a satis-  
factory foam on the galvanizing bath, it is, of  
course, impossible to proceed with the galvanizing  
operations. It is also observed that when exces-  
sive amounts of sulfates are present in zinc am-  
55 monium chloride fluxes, there is excessive "fum-  
ing". That is, the ammonium chloride in the flux

sublimes, rapidly destroying the efficacy of the  
flux.

Apparently the deleterious sulfates which ren-  
der zinc ammonium chloride fluxes unusable are  
inadvertently introduced into the flux in the 5  
course of manufacture or they are present be-  
cause the crude materials used are high in sul-  
fates. The sulfates are present, variously, as  
zinc sulfate, ammonium sulfate, lead sulfate, and  
even calcium sulfate. Inasmuch as it is the sul-  
10 fate radical which is deleterious, I have referred  
herein to the sulfate content in terms of the per-  
centage of  $SO_3$  found, in accordance with standard  
practice.

To render usable zinc ammonium chloride fluxes 15  
which contain excessive amounts of sulfates, it is  
only necessary to remove the sulfates in any de-  
sired manner. I have found it most satisfactory  
to remove so much of the sulfate as is necessary  
by adding an acid soluble barium salt, such as 20  
barium chloride or barium carbonate, to the flux  
while it is in dilute solution in the course of its  
manufacture. The resulting barium sulfate may  
be removed by decanting or filtering the solution.

Strangely enough, barium sulfate does not seem 25  
to exercise the deleterious effects experienced  
with most sulfates unless the barium sulfate is  
present in amounts exceeding about .5% as  $SO_3$ .  
If it is desired, therefore, to remove relatively 30  
small amounts of sulfate from concentrated zinc 35  
ammonium chloride liquors, the soluble barium  
salt may simply be added and the resulting  
barium sulfate included in the product. Of  
course, if this procedure is followed, great care  
must be exercised lest too large an amount of 40  
barium sulfate be present.

If the flux and foaming agent are to be added  
to a galvanizing bath indirectly by using the flux  
and foaming agent in a pre-dip, the excess of sul-  
fate may be removed by adding a soluble barium 45  
salt to the pre-dip. Here again, care must be  
exercised lest the barium sulfate content be too  
great.

Zinc ammonium chloride fluxes superior to those  
heretofore offered the trade may be prepared by 45  
removing substantially all of the sulfate content.  
If it is not expedient to remove all of the sul-  
fate, zinc ammonium chloride fluxes of very high  
quality may be prepared by treating the zinc 50  
ammonium chloride fluxes so that no more than 55  
about 0.1%  $SO_3$  is present. If it is found desirable  
to remove still less of the sulfate, satisfactory zinc  
ammonium chloride fluxes comparable to the best  
commercial fluxes heretofore offered the trade  
may be prepared by removing sulfate so that no 55

more than about 0.2%  $\text{SO}_3$  remains. It is not preferred, however, to leave as much as 0.2%  $\text{SO}_3$  in the flux because with this highest permissible  $\text{SO}_3$  content, it is ordinarily necessary to add a little more foaming agent than would be required with the fluxes having a lower  $\text{SO}_3$  content.

The following examples are given more fully to explain the practice of my invention.

*Example I*

10 A commercial zinc ammonium chloride galvanizing flux found unacceptable to the trade was analyzed and was found to contain 1.79% of sulfates computed as  $\text{SO}_3$ . This flux contained 15 soap bark as a foaming agent. When this flux was tried on a galvanizing bath, a foam formed very quickly, reaching a maximum thickness of about two inches, and subsiding after about four minutes. Using this flux, there was excessive 20 fuming. Following the teachings of this invention, the sulfates were removed from the flux by adding barium chloride to an aqueous solution thereof. Using the sulfate-free zinc ammonium chloride flux, a foam blanket about four and a half inches thick was obtained. This foam lasted 25 for about twenty four minutes, and there was very little fuming.

*Example II*

30 Another commercial zinc ammonium chloride flux found unacceptable to the trade was analyzed and was found to contain 0.36% of sulfate computed as  $\text{SO}_3$ . Testing this flux on a galvanizing pot, a foam about one inch thick and which lasted for only about two minutes was obtained. 35 Considerable fuming of the flux was observed, tho it was not quite as bad as the original flux mentioned in Example I. Following the procedure of this invention, the sulfates were removed from the flux by the use of barium chloride. The flux 40 then led to the production of a foam which lasted for about twenty two minutes and which was about four and a half inches thick.

*Example III*

45 A zinc ammonium chloride flux which was found unacceptable to the trade was analyzed and was found to contain 0.41% of sulfates computed as  $\text{SO}_3$ . This unsatisfactory flux produced a foam which lasted for about four minutes and 50 was about one inch thick. This flux contained 0.7% of glycerine as a foaming agent. To reduce the content of sulfates in the flux, there was added thereto a sulfate-free zinc ammonium chloride flux which contained 0.7% of glycerine. 55 The sulfate-free flux was added in an amount sufficient to bring the sulfate content of the mixture down to 0.05% computed as  $\text{SO}_3$ . The resulting mixture was used as a flux on a galvanizing pot and a foam which lasted for thirteen 60 minutes and which was about four inches thick

was obtained. Very little fuming was noted with the improved flux composition.

*Example IV*

A commercial zinc ammonium chloride flux 5 which contained 1.25% of soap bark as a foaming agent was analyzed and was treated to reduce the sulfate content to about 0.2% computed as  $\text{SO}_3$ . The flux was much improved, leading to the production of a foam which lasted for about six 10 minutes, and which was about one and one-half inches thick. There was moderate fuming. This flux was made more acceptable by increasing the soap bark content to 2.5% after which there was obtained a foam three inches thick which lasted 15 for fourteen minutes. The fuming was considerably lighter. It will be observed that at the upper limits of sulfate content specified by my invention, it is necessary to use a larger amount of foaming agents to produce entirely satisfactory 20 results. The use of an excess of a foaming agent is, of course, expensive and undesirable, and it is generally preferable, therefore, to reduce the sulfate content as much as possible.

*Example V*

A concentrated zinc ammonium chloride liquor 25 which contained sulfates equivalent to 0.5%  $\text{SO}_3$  was treated with barium chloride. The zinc ammonium chloride was crystallized from the solution and removed therefrom together with the barium sulfate. The flux thus produced was used 30 on a galvanizing pot and, after adding foaming agents in the customary amount, there was obtained a foam about two and a half inches thick 35 which lasted for about fourteen minutes. There was very little fuming. It is thus noted that barium sulfate equivalent to 0.5%  $\text{SO}_3$  does not exercise the deleterious effects observed with equally 40 large amounts of other sulfates. If barium sulfate be present in larger amounts, however, it adversely affects the characteristics of the flux.

While I have shown a number of specific procedures in the foregoing, it will readily be apparent that the sulfate content of zinc ammonium 45 chloride fluxes may be reduced in varying amounts and by various procedures without departing from the spirit of this invention.

I claim:

In a process for the treatment of a zinc ammonium chloride galvanizing flux which contains sulfates and hence is unsatisfactory by reason of the poor foam produced when it is used with foaming agents, the flux containing no more than about 0.5%  $\text{SO}_3$ , the steps comprising treating 55 the flux with a soluble barium compound to convert the sulfate to barium sulfate so that when used with foaming agents the flux will produce foams of satisfactory thickness and character.

RAYMOND J. KEPFER. 60